



US006030759A

# United States Patent [19]

Gula et al.

[11] Patent Number: 6,030,759

[45] Date of Patent: Feb. 29, 2000

[54] **COMPOSITE PHOTOGRAPHIC MATERIAL WITH LAMINATED BIAXIALLY ORIENTED POLYOLEFIN SHEETS WITH IMPROVED OPTICAL PERFORMANCE**

[75] Inventors: **Thaddeus S. Gula**, Rochester; **Peter T. Aylward**, Hilton; **Robert P. Bourdelais**, Pittsford; **Douglas N. Haydock**, Webster, all of N.Y.

[73] Assignee: **Eastman Kodak Company**, Rochester, N.Y.

[21] Appl. No.: **08/998,162**

[22] Filed: **Dec. 24, 1997**

[51] Int. Cl.<sup>7</sup> ..... **G03C 1/79**

[52] U.S. Cl. ..... **430/510**; 430/536; 430/538

[58] Field of Search ..... 430/536, 538, 430/510

## [56] References Cited

### U.S. PATENT DOCUMENTS

|           |         |                 |       |         |
|-----------|---------|-----------------|-------|---------|
| 4,187,113 | 2/1980  | Mathews et al.  | ..... | 430/538 |
| 4,283,486 | 8/1981  | Aono et al.     | ..... | 430/538 |
| 4,377,616 | 3/1983  | Ashcraft et al. | ..... |         |
| 4,632,869 | 12/1986 | Park et al.     | ..... |         |
| 4,758,462 | 7/1988  | Park et al.     | ..... |         |
| 4,912,333 | 3/1990  | Roberts et al.  | ..... |         |
| 4,994,312 | 2/1991  | Maier et al.    | ..... |         |
| 5,244,861 | 9/1993  | Campbell et al. | ..... | 430/201 |

|           |         |                   |       |         |
|-----------|---------|-------------------|-------|---------|
| 5,429,916 | 7/1995  | Ohshima           | ..... | 430/538 |
| 5,466,519 | 11/1995 | Shirakura et al.  | ..... | 430/538 |
| 5,476,708 | 12/1995 | Reed et al.       | ..... | 430/538 |
| 5,514,460 | 5/1996  | Surman et al.     | ..... |         |
| 5,866,282 | 2/1999  | Bourdelais et al. | ..... | 430/538 |

### FOREIGN PATENT DOCUMENTS

|              |         |                    |    |
|--------------|---------|--------------------|----|
| 0 582 750 A1 | 2/1994  | European Pat. Off. | .. |
| 0 643 328 A1 | 5/1995  | European Pat. Off. | .. |
| 0 662 633 A1 | 7/1995  | European Pat. Off. | .. |
| 0 803 377 A1 | 10/1997 | European Pat. Off. | .. |
| 1-282662     | 11/1989 | Japan              | .  |
| 4-256948     | 9/1992  | Japan              | .  |
| 2 325 750    | 12/1998 | United Kingdom     | .  |

Primary Examiner—Richard L. Schilling  
Attorney, Agent, or Firm—Paul A. Leipold

## [57] ABSTRACT

The invention relates to a photographic element comprising a paper base, at least one photosensitive silver halide layer, a layer of microvoided polymer sheet between said paper base and said silver halide layer, and one or more other non-voided layers between said silver halide layer and said microvoided layer, and one or more other non-voided layers between said microvoided layer and said paper base.

The voided or non-voided layers have levels of TiO<sub>2</sub> and colorants adjusted to provide optimum optical properties for control of MTF, LSTAR, and OPACITY.

**20 Claims, No Drawings**

**COMPOSITE PHOTOGRAPHIC MATERIAL  
WITH LAMINATED BIAXIALLY ORIENTED  
POLYOLEFIN SHEETS WITH IMPROVED  
OPTICAL PERFORMANCE**

**FIELD OF THE INVENTION**

This invention relates to photographic materials. In a preferred form it relates to base materials for photographic color papers.

**BACKGROUND OF THE INVENTION**

In the formation of color paper it is known that the base paper has applied thereto a layer of polymer, typically polyethylene. This layer serves to provide waterproofing to the paper, as well as providing a smooth surface on which the photosensitive layers are formed. The formation of a suitably smooth surface is difficult requiring great care and expense to ensure proper laydown and cooling of the polyethylene layers. One defect in prior formation techniques is caused when an air bubble is trapped between the forming roller and the polyethylene which will form the surface for casting of photosensitive materials. This air bubble will form a pit that will cause a defect in the photographic performance of photographic materials formed on the polyethylene. It would be desirable if a more reliable and improved surface could be formed at less expense.

In color papers there is a need for providing color papers with improved resistance to curl. Present color papers will curl during development and storage. Such curl is thought to be caused by the different properties of the layers of the color paper as it is subjected to the developing and drying processes. Humidity changes during storage of color photographs lead to curling. There are particular problems with color papers when they are subjected to extended high humidity storage such as at greater than 50% relative humidity. Extremely low humidity of less than 20% relative humidity also will cause photographic papers to curl.

In photographic papers the polyethylene layer also serves as a carrier layer for titanium dioxide and other whitener materials as well as tint materials. It would be desirable if the colorant materials rather than being dispersed throughout the polyethylene layer could be concentrated nearer the surface of the layer where they would be more effective photographically.

While prior art photographic materials have been satisfactory, there is a need for images that can more closely replicate the actual scenes photographed.

One improvement would be sharpness, or the ability to replicate fine details of the image. This can be measured by mathematical calculations, one such method is called the MTF or Modulation Transfer Function. In this test, a fine repeating sinusoidal pattern of photographic density variation near the resolution of the human eye is exposed on a photographic print, when the print is developed the resulting density variation is compared to the expected density and a ratio is obtained to determine the magnitude of the transfer coefficient at that frequency. A number of 100 denotes perfect replication, and this number is relatively easy to obtain at spatial frequencies of 0.2 cycle/mm. At a finer spacing of 2.0 cycles/mm typical color photographic prints have a 70 rating or 70% replication.

Another improvement desired would be the visual appearance of whiteness in exposed subject areas like snow or a wedding gown. Because of imperfect light reflection from the surface underneath the image bearing emulsion, the

current photographic prints tend to look yellow, and if corrections to the surface are made, then they may appear gray or blue. The measurement for this problem is a DMIN value which is a measurement of the photographic minimum density attained on a specially exposed print. In practice, it has been found that the surface under the silver halide layer can be measured to predict DMIN by using the L Star UVO value. The L Star UVO (ultraviolet filter out) can be obtained from a HUNTER spectrophotometer, CIE system, using procedure D65.

Improvements in another optical property affected by the base paper is opacity, or the ability of the photographic element to hide any visual evidence of what is behind the print. For example, the logo printed on the back, or the outline of the shadow of the fingers holding the print. Opacity numbers are generated by taking the ratio of the light reflected from the viewing surface of a generally white image when it is backed by a white background and then backed by a black background. A ratio of 1, which is reported as 100, is perfect. Most photographic materials today are rated at 92 to 95.

It would be particularly desirable if there was a way to produce improvements in MTF, LSTAR, and OPACITY at the same time.

Prior art photographic materials have suggested monolayer or coextruded layer coatings on raw base that are thicker and/or more concentrated with titanium dioxide ( $TiO_2$ ) and colorants. Other high refractive index materials like zinc oxide or other finely divided solids are also used. In general, these improvements are costly and processing and coating these concentrated layers create manufacturing problems with specks, lines and surface disruptions. The highly loaded layers deteriorate the strength property of the coatings and may be involved with poor adhesion to the base paper or to the image bearing emulsion layer. Also, the coating speed of these layers may be lower.

The details of an invention and a description of the problems encountered with highly loaded coextruded layers is recorded in U.S. Pat. No. 5,466,519.

It has been proposed in U.S. Pat. No. 5,244,861 to utilize biaxially oriented polypropylene in receiver sheets for thermal dye transfer. As will be shown, these materials appear to have very unique abilities to optimize thin layers for improved optical performance.

**PROBLEM TO BE SOLVED BY THE  
INVENTION**

There remains a need for a more effective layer between the photosensitive layers and the base paper to more effectively carry colorant materials so that we may create major improvements in all three optical performance properties (MTF, LSTAR, and OPACITY) that are practical, manufacturable, and cost effective.

**SUMMARY OF THE INVENTION**

An object of the invention is to provide improved photographic papers.

It is an object of the invention to provide photographic images that have improved image reproduction.

It is another object of the invention to reduce the amount of pigments or tinting agents used in the prior art.

It is another object of the invention to provide photographic elements that can be easily manufactured without adhesion, lines, spots or other physical properties.

It is another object of the invention to provide photographic elements that can be coated at very high speed.

It is another object of the invention to provide a way to recycle any appropriate off cuts or scraps of the extruded coatings in a way that does not affect the optical properties of a photographic element.

These and other objects of the invention are generally accomplished by providing a photographic element comprising a paper base, at least one photosensitive silver halide layer, a layer of biaxially oriented polyolefin sheet between said paper base and said silver halide layer, wherein said biaxially oriented polyolefin sheet comprises an upper layer that comprises between 4 and 24% of a white pigment; and adjacent said upper layer a core layer that is microvoiced; and adjacent and below said core layer a layer of polyolefin that is substantially colorant and pigment free.

#### ADVANTAGEOUS EFFECT OF THE INVENTION

The invention provides an improved base for casting of photosensitive layers. It particularly provides improved base for color photographic materials that have improved images.

#### DETAILED DESCRIPTION OF THE INVENTION

There are numerous advantages of the invention over prior practices in the art. The invention provides a photographic element that has much less tendency to curl when exposed to extremes of humidity. Further, the invention provides a photographic paper that is much lower in cost as the criticalities of the formation of the polyethylene are removed. There is no need for the difficult and expensive casting and cooling in forming a surface on the polyethylene layer as the biaxially oriented polymer sheet of the invention provides a high quality surface for casting of photosensitive layers. Photographic materials utilizing microvoiced sheets of the invention have improved resistance to tearing. The photographic materials of the invention are lower in cost to produce as the microvoiced sheet may be scanned for quality prior to assembly into the photographic member. With present polyethylene layers the quality of the layer cannot be assessed until after complete formation of the base paper with the polyethylene waterproofing layer attached. Therefore, any defects result in expensive discard of expensive product. The invention allows faster hardening of photographic paper emulsion, as water vapor is not transmitted from the emulsion through the biaxially oriented sheets.

Another advantage of the microvoiced sheets of the invention is that they are more opaque than titanium dioxide loaded polyethylene of present products. They achieve this opacity partly by the use of the voids. The photographic elements of this invention are more scratch resistant as the oriented polymer sheet on the back of the photographic element resists scratching and other damage more readily than polyethylene. These and other advantages will be apparent from the detailed description below.

The terms as used herein, "top", "upper", "emulsion side", and "face" mean the side or toward the side of a photographic member bearing the imaging layers. The terms "bottom", "lower side", and "back" mean the side or toward the side of the photographic member opposite from the side bearing the photosensitive imaging layers or developed image.

Any suitable biaxially oriented polyolefin sheet with an outer white pigment layer may be utilized in the invention for the sheet on the top side of the laminated base of the invention. Microvoiced composite biaxially oriented sheets

are preferred and are conveniently manufactured by coextrusion of the core and surface layers, followed by biaxial orientation, whereby voids are formed around void-initiating material contained in the core layer. Such composite sheets are disclosed in, for example, U.S. Pat. Nos. 4,377,616; 4,758,462 and 4,632,869, the disclosure of which is incorporated by reference.

The density (specific gravity) of the composite sheet, expressed in terms of "percent of solid density" is calculated as follows:

$$\text{Composite Sheet Density}/\text{Polymer Density} \times 100 = \% \text{ of Solid Density}$$

should be between 45% and 100%, preferably between 67% and 100%. As the percent solid density becomes less than 67%, the composite sheet becomes less manufacturable due to a drop in tensile strength and it becomes more susceptible to physical damage.

The thickness of the core layer is preferably between 10 and 60  $\mu\text{m}$ . Manufacturing a voided layer less than 10  $\mu\text{m}$  is very difficult. Above 60  $\mu\text{m}$ , the structure becomes more susceptible to physical damage caused by stresses encountered when the photographic element is bent. Such stresses are encountered when photographic images are viewed and handled by the consumer.

The thickness of the upper layer (the layer between the photosensitive layer and the voided layer) is preferably between 1 and 15  $\mu\text{m}$ . Below 1  $\mu\text{m}$  in thickness, the microvoiced sheet becomes difficult to manufacture as the limits of a biaxially oriented layer are reached. Above 15  $\mu\text{m}$ , little improvement is seen in the optical performance of the layer.

The thickness of the layer adjacent and below the microvoiced layer is preferably between 2 and 15  $\mu\text{m}$ . For the same reasons manufacturing outside this range can either cause manufacturing problems or does not improve the optical performance of the photographic support.

The total thickness of the composite sheet can range from 12 to 100  $\mu\text{m}$ , preferably from 20 to 70  $\mu\text{m}$ . Below 20  $\mu\text{m}$ , the microvoiced sheets may not be thick enough to minimize any inherent non-planarity in the support and would be more difficult to manufacture. At thickness higher than 70  $\mu\text{m}$ , little improvement in either surface smoothness or mechanical properties are seen, and so there is little justification for the further increase in cost for extra materials.

The biaxially oriented sheets of the invention preferably have a water vapor permeability that is less than  $0.85 \times 10^{-5}$  g/mm<sup>2</sup>/day. This allows faster emulsion hardening, as the laminated support of this invention does not transmit water vapor from the emulsion layers during coating of the emulsions on the support. The transmission rate is measured by ASTM F1249.

"Void" is used herein to mean devoid of added solid and liquid matter, although it is likely the "voids" contain gas. The void-initiating particles which remain in the finished packaging sheet core should be from 0.1 to 10  $\mu\text{m}$  in diameter, preferably round in shape, to produce voids of the desired shape and size. The size of the void is also dependent on the degree of orientation in the machine and transverse directions. Ideally, the void would assume a shape which is defined by two opposed and edge contacting concave disks.

In other words, the voids tend to have a lens-like or biconvex shape. The voids are oriented so that the two major dimensions are aligned with the machine and transverse directions of the sheet. The Z-direction axis is a minor dimension and is roughly the size of the cross diameter of the voiding particle. The voids generally tend to be closed cells, and thus there is virtually no path open from one side of the voided core to the other side through which gas or liquid can traverse.

The void-initiating material may be selected from a variety of materials, and should be present in an amount of about 5–50% by weight based on the weight of the core matrix polymer. Preferably, the void-initiating material comprises a polymeric material. When a polymeric material is used, it may be a polymer that can be melt-mixed with the polymer from which the core matrix is made and be able to form dispersed spherical particles as the suspension is cooled down. Examples of this would include nylon dispersed in polypropylene, polybutylene terephthalate in polypropylene, or polypropylene dispersed in polyethylene terephthalate. If the polymer is preshaped and blended into the matrix polymer, the important characteristic is the size and shape of the particles. Spheres are preferred and they can be hollow or solid. These spheres may be made from cross-linked polymers which are members selected from the group consisting of an alkenyl aromatic compound having the general formula  $\text{Ar}-\text{C}(\text{R})=\text{CH}_2$ , wherein Ar represents an aromatic hydrocarbon radical, or an aromatic halohydrocarbon radical of the benzene series and R is hydrogen or the methyl radical; acrylate-type monomers include monomers of the formula  $\text{CH}_2=\text{C}(\text{R}')-\text{C}(\text{O})(\text{OR})$  wherein R is selected from the group consisting of hydrogen and an alkyl radical containing from about 1 to 12 carbon atoms and R' is selected from the group consisting of hydrogen and methyl; copolymers of vinyl chloride and vinylidene chloride, acrylonitrile and vinyl chloride, vinyl bromide, vinyl esters having formula  $\text{CH}_2=\text{CH}(\text{O})\text{COR}$ , wherein R is an alkyl radical containing from 2 to 18 carbon atoms; acrylic acid, methacrylic acid, itaconic acid, citraconic acid, maleic acid, fumaric acid, oleic acid, vinylbenzoic acid; the synthetic polyester resins which are prepared by reacting terephthalic acid and dialkyl terephthalates or ester-forming derivatives thereof, with a glycol of the series  $\text{HO}(\text{CH}_2)_n\text{OH}$  wherein n is a whole number within the range of 2–10 and having reactive olefinic linkages within the polymer molecule, the above described polyesters which include copolymerized therein up to 20 percent by weight of a second acid or ester thereof having reactive olefinic unsaturation and mixtures thereof, and a cross-linking agent selected from the group consisting of divinylbenzene, diethylene glycol dimethacrylate, diallyl fumarate, diallyl phthalate and mixtures thereof.

Examples of typical monomers for making the crosslinked polymer include styrene, butyl acrylate, acrylamide, acrylonitrile, methyl methacrylate, ethylene glycol dimethacrylate, vinyl pyridine, vinyl acetate, methyl acrylate, vinylbenzyl chloride, vinylidene chloride, acrylic acid, divinylbenzene, acrylamidomethylpropane sulfonic acid, vinyl toluene, etc. Preferably, the cross-linked polymer is polystyrene or poly(methyl methacrylate). Most preferably, it is polystyrene and the cross-linking agent is divinylbenzene.

Processes well known in the art yield non-uniformly sized particles, characterized by broad particle size distributions. The resulting beads can be classified by screening the beads spanning the range of the original distribution of sizes. Other processes such as suspension polymerization, limited coalescence, directly yield very uniformly sized particles.

The void-initiating materials may be coated with a agents to facilitate voiding. Suitable agents or lubricants include colloidal silica, colloidal alumina, and metal oxides such as tin oxide and aluminum oxide. The preferred agents are colloidal silica and alumina, most preferably, silica. The cross-linked polymer having a coating of an agent may be prepared by procedures well known in the art. For example, conventional suspension polymerization processes wherein

the agent is added to the suspension is preferred. As the agent, colloidal silica is preferred.

The void-initiating particles can also be inorganic spheres, including solid or hollow glass spheres, metal or ceramic beads or inorganic particles such as clay, talc, barium sulfate, calcium carbonate. The important thing is that the material does not chemically react with the core matrix polymer to cause one or more of the following problems: (a) alteration of the crystallization kinetics of the matrix polymer, making it difficult to orient, (b) destruction of the core matrix polymer, (c) destruction of the void-initiating particles, (d) adhesion of the void-initiating particles to the matrix polymer, or (e) generation of undesirable reaction products, such as toxic or high color moieties. The void-initiating material should not be photographically active or degrade the performance of the photographic element in which the biaxially oriented polyolefin film is utilized.

For the biaxially oriented sheets on the top side toward the emulsion, suitable classes of thermoplastic polymers for the biaxially oriented sheet and the core matrix-polymer of the preferred composite sheet comprise polyolefins.

Suitable polyolefins include polypropylene, polyethylene, polymethylpentene, polystyrene, polybutylene and mixtures thereof. Polyolefin copolymers, including copolymers of propylene and ethylene such as hexene, butene, and octene are also useful. Polypropylene is preferred, as it is low in cost and has desirable strength properties.

The nonvoided skin layers of the composite sheet can be made of the same polymeric materials as listed above for the core matrix. The composite sheet can be made with skin(s) of the same polymeric material as the core matrix, or it can be made with skin(s) of different polymeric composition than the core matrix. For compatibility, an auxiliary layer can be used to promote adhesion of the skin layer to the core.

Addenda may be added to the core matrix and/or to the skins to improve the optical properties of the photographic support. Titanium dioxide is preferred and is used in this invention to improve image sharpness or MTF, opacity and whiteness. The  $\text{TiO}_2$  used may be either anatase or rutile type. In the case of whiteness, anatase is the preferred type. In the case of sharpness, rutile is the preferred. Further, both anatase and rutile  $\text{TiO}_2$  may be blended to improve both whiteness and sharpness. Examples of  $\text{TiO}_2$  that are acceptable for a photographic system are Dupont Chemical Co. R101 rutile  $\text{TiO}_2$  and DuPont Chemical Co. R104 rutile  $\text{TiO}_2$ . Other pigments known in the art to improve photographic optical responses may also be used in this invention. Preferred pigments are talc, kaolin,  $\text{CaCO}_3$ ,  $\text{BaSO}_4$ ,  $\text{ZnO}$ ,  $\text{TiO}_2$ ,  $\text{ZnS}$ , and  $\text{MgCO}_3$ .

The preferred weight percent of white pigment to be added to the biaxially oriented layers between the photo-sensitive layer and the voided layer can range from 4% and 24% by weight, preferably from 15% to 20% of the weight of the polymer in that layer. Below 15% the optical properties of the voided biaxially oriented sheet do not show a significant improvement over prior art photographic paper. Above 20%, manufacturing problems such as unwanted voiding and a loss of coating speed are encountered. The voided layer may also contain white pigments. The voided layer may contain between 2 and 18% white pigment based on the weight of the polymer in that layer, preferably between 2% and 8%. Below 2%, the optical properties of the voided biaxially oriented sheet do not show a significant improvement. Above 8%, the voided layer suffers from a loss in mechanical strength which will reduce the commercial value of the photographic support of this invention as images are handled and viewed by consumers.

The layer adjacent and below the voided layer may also contain white pigments of this invention. A layer that is substantially colorant and pigment free are preferred as there is little improvement in the optical performance of the photographic support when colorants and white pigments are added below the voided layer.

The upper most layer or the upper surface of the biaxially oriented sheet may also contain white pigments. A layer that is substantially white pigment free is preferred as there is little improvement in the optical performance of the photographic support and there exists several melt extrusion manufacturing problems such as die lines and spots when the skin layer contains white pigments.

Additional addenda may be added to the core matrix and/or to the skins to improve the optical properties such as image sharpness, opacity and whiteness of these sheets. This would also include adding fluorescing agents which absorb energy in the UV region and emit light largely in the blue region, or other additives which would improve the physical properties of the sheet or the manufacturability of the sheet.

The coextrusion, quenching, orienting, and heat setting of these composite sheets may be effected by any process which is known in the art for producing oriented sheet, such as by a flat sheet process or a bubble or tubular process. The flat sheet process involves extruding the blend through a slit die and rapidly quenching the extruded web upon a chilled casting drum so that the corematrix polymer component of the sheet and the skin component(s) are quenched below their glass solidification temperature. The quenched sheet is then biaxially oriented by stretching in mutually perpendicular directions at a temperature above the glass transition temperature, below the melting temperature of the matrix polymers. The sheet may be stretched in one direction and then in a second direction or may be simultaneously stretched in both directions. After the sheet has been stretched, it is heat set by heating to a temperature sufficient to crystallize or anneal the polymers while restraining to some degree the sheet against retraction in both directions of stretching.

The composite sheet, while described as having preferably at least three layers of a microvoided core and a skin layer on each side, may also be provided with additional layers that may serve to change the properties of the biaxially oriented sheet. Biaxially oriented sheets could be formed with surface layers that would provide an improved adhesion, or look to the support and photographic element. The biaxially oriented extrusion could be carried out with as many as 10 layers if desired to achieve some particular desired property.

These composite sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photo sensitive layers. Examples of this would be acrylic coatings for printability, coating polyvinylidene chloride for heat seal properties. Further examples include flame, plasma or corona discharge treatment to improve printability or adhesion.

By having at least one nonvoided skin on the microvoided core, the tensile strength of the sheet is increased and makes it more manufacturable. It allows the sheets to be made at wider widths and higher draw ratios than when sheets are made with all layers voided. Coextruding the layers further simplifies the manufacturing process.

The structure of a typical biaxially oriented, microvoided sheet of the invention is as follows:

---

|   |                                                                |
|---|----------------------------------------------------------------|
| 5 | solid skin layer<br>microvoided core layer<br>solid skin layer |
|---|----------------------------------------------------------------|

---

The sheet on the side of the base paper opposite to the emulsion layers may be any suitable sheet. The sheet may or may not be microvoided. It may have the same composition as the sheet on the top side of the paper backing material. Biaxially oriented sheets are conveniently manufactured by coextrusion of the sheet, which may contain several layers, followed by biaxial orientation. Such biaxially oriented sheets are disclosed in, for example, U.S. Pat. No. 4,764,425.

The preferred biaxially oriented sheet is a biaxially oriented polyolefin sheet, most preferably a sheet of polyethylene or polypropylene. The thickness of the biaxially oriented sheet should be from 10 to 150  $\mu\text{m}$ . Below 15  $\mu\text{m}$ , the sheets may not be thick enough to minimize any inherent non-planarity in the support and would be more difficult to manufacture. At thicknesses higher than 70  $\mu\text{m}$ , little improvement in either surface smoothness or mechanical properties are seen, and so there is little justification for the further increase in cost for extra materials.

Suitable classes of thermoplastic polymers for the biaxially oriented sheet include polyolefins, polyesters, polyamides, polycarbonates, cellulosic esters, polystyrene, polyvinyl resins, polysulfonamides, polyethers, polyimides, polyvinylidene fluoride, polyurethanes, polyphenylenesulfides, polytetrafluoroethylene, polyacetals, polysulfonates, polyester ionomers, and polyolefin ionomers. Copolymers and/or mixtures of these polymers can be used.

Suitable polyolefins include polypropylene, polyethylene, polymethylpentene, and mixtures thereof. Polyolefin copolymers, including copolymers of propylene and ethylene such as hexene, butene and octene are also useful. Polypropylenes are preferred because they are low in cost and have good strength and surface properties.

Suitable polyesters include those produced from aromatic, aliphatic or cycloaliphatic dicarboxylic acids of 4–20 carbon atoms and aliphatic or alicyclic glycols having from 2–24 carbon atoms. Examples of suitable dicarboxylic acids include terephthalic, isophthalic, phthalic, naphthalene dicarboxylic acid, succinic, glutaric, adipic, azelaic, sebacic, fumaric, maleic, itaconic, 1,4-cyclohexanedicarboxylic, sodiosulfoisophthalic and mixtures thereof. Examples of suitable glycols include ethylene glycol, propylene glycol, butanediol, pentanediol, hexanediol, 1,4-cyclohexanedimethanol, diethylene glycol, other polyethylene glycols and mixtures thereof. Such polyesters are well known in the art and may be produced by well known techniques, e.g., those described in U.S. Pat. No. 2,465,319 and U.S. Pat. No. 2,901,466. Preferred continuous matrix polyesters are those having repeat units from terephthalic acid or naphthalene dicarboxylic acid and at least one glycol selected from ethylene glycol, 1,4-butanediol and 1,4-cyclohexanedimethanol. Poly(ethylene terephthalate), which may be modified by small amounts of other monomers, is especially preferred. Other suitable polyesters include liquid crystal copolymers formed by the inclusion of suitable amount of a co-acid component such as stilbene dicarboxylic acid. Examples of such liquid crystal copolymers are those disclosed in U.S. Pat. Nos. 4,420,607; 4,459,402; and 4,468,510.

Useful polyamides include nylon 6, nylon 66, and mixtures thereof. Copolymers of polyamides are also suitable continuous phase polymers. An example of a useful polycarbonate is bisphenol-A polycarbonate. Cellulosic esters suitable for use as the continuous phase polymer of the composite sheets include cellulose nitrate, cellulose triacetate, cellulose diacetate, cellulose acetate propionate, cellulose acetate butyrate, and mixtures or copolymers thereof. Useful polyvinyl resins include polyvinyl chloride, poly(vinyl acetal), and mixtures thereof. Copolymers of vinyl resins can also be utilized.

The biaxially oriented sheet on the back side of the laminated base can be made with layers of the same polymeric material, or it can be made with layers of different polymeric composition. For compatibility, an auxiliary layer can be used to promote adhesion of multiple layers.

Addenda may be added to the biaxially oriented sheet to improve the whiteness of these sheets. This would include any process which is known in the art including adding a white pigment, such as titanium dioxide, barium sulfate, clay, or calcium carbonate. This would also include adding fluorescing agents which absorb energy in the UV region and emit light largely in the blue region, or other additives which would improve the physical properties of the sheet or the manufacturability of the sheet.

The coextrusion, quenching, orienting, and heat setting of these biaxially oriented sheets may be effected by any process which is known in the art for producing oriented sheet, such as by a flat sheet process or a bubble or tubular process. The flat sheet process involves extruding or coextruding the blend through a slit die and rapidly quenching the extruded or coextruded web upon a chilled casting drum so that the polymer component(s) of the sheet are quenched below their solidification temperature. The quenched sheet is then biaxially oriented by stretching in mutually perpendicular directions at a temperature above the glass transition temperature of the polymer(s). The sheet may be stretched in one direction and then in a second direction or may be simultaneously stretched in both directions. After the sheet has been stretched, it is heat set by heating to a temperature sufficient to crystallize the polymers while restraining to some degree the sheet against retraction in both directions of stretching.

The biaxially oriented sheet on the back side of the laminated base, while described as having preferably at least one layer, may also be provided with additional layers that may serve to change the properties of the biaxially oriented sheet. A different effect may be achieved by additional layers. Such layers might contain tints, antistatic materials, or slip agents to produce sheets of unique properties. Biaxially oriented sheets could be formed with surface layers that would provide an improved adhesion, or look to the support and photographic element. The biaxially oriented extrusion could be carried out with as many as 10 layers if desired to achieve some particular desired property.

These biaxially oriented sheets may be coated or treated after the coextrusion and orienting process or between casting and full orientation with any number of coatings which may be used to improve the properties of the sheets including printability, to provide a vapor barrier, to make them heat sealable, or to improve the adhesion to the support or to the photo sensitive layers. Examples of this would be acrylic coatings for printability, coating polyvinylidene chloride for heat seal properties. Further examples include flame, plasma or corona discharge treatment to improve printability or adhesion.

The structure of a typical biaxially oriented sheet that may be laminated to the backside with the treated skin layer on the outside of the package is as follows:



The support to which the microvoided composite sheets and biaxially oriented sheets are laminated for the laminated support of the photosensitive silver halide layer may be a polymeric, a synthetic paper, cloth, woven polymer fibers, or a cellulose fiber paper support, or laminates thereof. The base also may be a microvoided polyethylene terephthalate such as disclosed in U.S. Pat. Nos. 4,912,333; 4,994,312; and 5,055,371, the disclosure of which is incorporated by reference.

The preferred support is a photographic grade cellulose fiber paper. When using a cellulose fiber paper support, it is preferable to extrusion laminate the microvoided composite sheets to the base paper using a polyolefin resin. Extrusion laminating is carried out by bringing together the biaxially oriented sheets of the invention and the base paper with application of an adhesive between them followed by their being pressed in a nip such as between two rollers. The adhesive may be applied to either the biaxially oriented sheets or the base paper prior to their being brought into the nip. In a preferred form the adhesive is applied into the nip simultaneously with the biaxially oriented sheets and the base paper. The adhesive may be any suitable material that does not have a harmful effect upon the photographic element. A preferred material is polyethylene that is melted at the time it is placed into the nip between the paper and the biaxially oriented sheet. Addenda may also be added to the adhesive layer. Any known material used in the art to improve the optical performance of the system may be used. The use of TiO<sub>2</sub> is preferred.

During the lamination process, it is desirable to maintain control of the tension of the biaxially oriented sheet(s) in order to minimize curl in the resulting laminated receiver support. For high humidity applications (>50% RH) and low humidity applications (<20% RH), it is desirable to laminate both a front side and back side film to keep curl to a minimum.

In one preferred embodiment, in order to produce photographic elements with a desirable photographic look and feel, it is preferable to use relatively thick paper supports (e.g., at least 120 mm thick, preferably from 120 to 250 mm thick) and relatively thin microvoided composite packaging films (e.g., less than 50 mm thick, preferably from 20 to 50 mm thick, more preferably from 30 to 50 mm thick).

The photographic elements can be single color elements or multicolor elements. Multicolor elements contain image dye-forming units sensitive to each of the three primary regions of the spectrum. Each unit can comprise a single emulsion layer or multiple emulsion layers sensitive to a given region of the spectrum. The layers of the element, including the layers of the image-forming units, can be arranged in various orders as known in the art. In an alternative format, the emulsions sensitive to each of the three primary regions of the spectrum can be disposed as a single segmented layer.

The photographic emulsions useful for this invention are generally prepared by precipitating silver halide crystals in a colloidal matrix by methods conventional in the art. The colloid is typically a hydrophilic film forming agent such as gelatin, alginic acid, or derivatives thereof.

The crystals formed in the precipitation step are washed and then chemically and spectrally sensitized by adding

## 11

spectral sensitizing dyes and chemical sensitizers, and by providing a heating step during which the emulsion temperature is raised, typically from 40° C. to 70° C., and maintained for a period of time. The precipitation and spectral and chemical sensitization methods utilized in preparing the emulsions employed in the invention can be those methods known in the art.

Chemical sensitization of the emulsion typically employs sensitizers such as: sulfur-containing compounds, e.g., allyl isothiocyanate, sodium thiosulfate and allyl thiourea; reducing agents, e.g., polyamines and stannous salts; noble metal compounds, e.g., gold, platinum; and polymeric agents, e.g., polyalkylene oxides. As described, heat treatment is employed to complete chemical sensitization. Spectral sensitization is effected with a combination of dyes, which are designed for the wavelength range of interest within the visible or infrared spectrum. It is known to add such dyes both before and after heat treatment.

After spectral sensitization, the emulsion is coated on a support. Various coating techniques include dip coating, air knife coating, curtain coating and extrusion coating.

The silver halide emulsions utilized in this invention may be comprised of any halide distribution. Thus, they may be comprised of silver chloride, silver bromide, silver bromochloride, silver chlorobromide, silver iodochloride, silver iodobromide, silver bromoiodochloride, silver chloroiodobromide, silver iodobromochloride, and silver iodochlorobromide emulsions. It is preferred, however, that the emulsions be predominantly silver chloride emulsions. By predominantly silver chloride, it is meant that the grains of the emulsion are greater than about 50 mole percent silver chloride. Preferably, they are greater than about 90 mole percent silver chloride; and optimally greater than about 95 mole percent silver chloride.

The silver halide emulsions can contain grains of any size and morphology. Thus, the grains may take the form of cubes, octahedrons, cubooctahedrons, or any of the other naturally occurring morphologies of cubic lattice type silver halide grains. Further, the grains may be irregular such as spherical grains or tabular grains. Grains having a tabular or cubic morphology are preferred.

The photographic elements of the invention may utilize emulsions as described in *The Theory of the Photographic Process*, Fourth Edition, T. H. James, Macmillan Publishing Company, Inc., 1977, pages 151-152. Reduction sensitization has been known to improve the photographic sensitivity of silver halide emulsions. While reduction sensitized silver halide emulsions generally exhibit good photographic speed, they often suffer from undesirable fog and poor storage stability.

Reduction sensitization can be performed intentionally by adding reduction sensitizers, chemicals which reduce silver ions to form metallic silver atoms, or by providing a reducing environment such as high pH (excess hydroxide ion) and/or low pAg (excess silver ion). During precipitation of a silver halide emulsion, unintentional reduction sensitization can occur when, for example, silver nitrate or alkali solutions are added rapidly or with poor mixing to form emulsion grains. Also, precipitation of silver halide emulsions in the presence of ripeners (grain growth modifiers) such as thioethers, selenoethers, thioureas, or ammonia tends to facilitate reduction sensitization.

Examples of reduction sensitizers and environments which may be used during precipitation or spectral/chemical sensitization to reduction sensitized an emulsion include ascorbic acid derivatives; tin compounds; polyamine compounds; and thiourea dioxide-based compounds described in

## 12

U.S. Pat. Nos. 2,487,850; 2,512,925; and British Patent 789,823. Specific examples of reduction sensitizers or conditions, such as dimethylamineborane, stannous chloride, hydrazine, high pH (pH 8-11) and low pAg (pAg 5 1-7) ripening are discussed by S. Collier in *Photographic Science and Engineering*, 23,113 (1979). Examples of processes for preparing intentionally reduction sensitized silver halide emulsions are described in EP 0 348934 A1 (Yamashita), EP 0 369491 (Yamashita), EP 0 371388 (Ohashi), EP 0 396424 A1 (Takada), EP 0 404142 A1 (Yamada), and EP 0 435355 A1 (Makino).

The photographic elements of this invention may use emulsions doped with Group VIII metals such as iridium, rhodium, osmium, and iron as described in *Research Disclosure*, September 1994, Item 36544, Section I, published by Kenneth Mason Publications, Ltd., Dudley Annex, 12a North Street, Emsworth, Hampshire PO10 7DQ, ENGLAND. Additionally, a general summary of the use of iridium in the sensitization of silver halide emulsions is contained in Carroll, "Iridium Sensitization: A Literature Review," *Photographic Science and Engineering*, Vol. 24, No. 6, 1980. A method of manufacturing a silver halide emulsion by chemically sensitizing the emulsion in the presence of an iridium salt and a photographic spectral sensitizing dye is described in U.S. Pat. No. 4,693,965. In some cases, when such dopants are incorporated, emulsions show an increased fresh fog and a lower contrast sensitometric curve when processed in the color reversal E-6 process as described in *The British Journal of Photography Annual*, 1982, pages 201-203.

A typical multicolor photographic element of the invention comprises the invention laminated support bearing a cyan dye image-forming unit comprising at least one red-sensitive silver halide emulsion layer having associated therewith at least one cyan dye-forming coupler; a magenta image-forming unit comprising at least one green-sensitive silver halide emulsion layer having associated therewith at least one magenta dye-forming coupler; and a yellow dye image-forming unit comprising at least one blue-sensitive silver halide emulsion layer having associated therewith at least one yellow dye-forming coupler. The element may contain additional layers, such as filter layers, interlayers, overcoat layers, subbing layers, and the like. The support of the invention may also be utilized for black and white photographic print elements.

The photographic elements may also contain a transparent magnetic recording layer such as a layer containing magnetic particles on the underside of a transparent support, as in U.S. Pat. Nos. 4,279,945 and 4,302,523. Typically, the element will have a total thickness (excluding the support) of from about 5 to about 30  $\mu\text{m}$ .

In the following Table, reference will be made to (1) *Research Disclosure*, December 1978, Item 17643, (2) *Research Disclosure*, December 1989, Item 308119, and (3) *Research Disclosure*, September 1994, Item 36544, all published by Kenneth Mason Publications, Ltd., Dudley Annex, 12a North Street, Emsworth, Hampshire PO10 7DQ, ENGLAND. The Table and the references cited in the Table are to be read as describing particular components suitable for use in the elements of the invention. The Table and its cited references also describe suitable ways of preparing, exposing, processing and manipulating the elements, and the images contained therein.

| Reference | Section                        | Subject Matter                                                                    |
|-----------|--------------------------------|-----------------------------------------------------------------------------------|
| 1         | I, II                          | Grain composition, morphology and preparation                                     |
| 2         | I, II, IX, X, XI, XII, XIV, XV | Emulsion preparation including hardeners, coating aids, addenda, etc.             |
| 3         | I, II, III, IX A & B           | Chemical sensitization and spectral sensitization/desensitization                 |
| 1         | III, IV                        | UV dyes, optical brighteners, luminescent dyes                                    |
| 2         | IV, V                          | VI                                                                                |
| 3         | V                              | Antifoggants and stabilizers                                                      |
| 2         | VI                             | VII                                                                               |
| 3         | VIII                           | Absorbing and scattering materials; Antistatic layers; matting agents             |
| 2         | VIII, XIII, XVI                | VIII, IX C & D                                                                    |
| 3         | XVI                            | Image-couplers and image-modifying couplers; Dye stabilizers and hue modifiers    |
| 1         | XVII                           | Supports                                                                          |
| 2         | XVII                           | XV                                                                                |
| 3         | XV                             | XI                                                                                |
| 3         | XII, XIII                      | Specific layer arrangements Negative working emulsions; Direct positive emulsions |
| 2         | XVIII                          | Exposure                                                                          |
| 3         | XVI                            | XIX, XX                                                                           |
| 1         | XIX, XX                        | Chemical processing; Developing agents                                            |
| 2         | XIX, XX, XXII                  | XVIII, XIX, XX                                                                    |
| 3         | XVIII, XIX, XX                 | XIV                                                                               |
| 3         | XIV                            | Scanning and digital processing procedures                                        |

The photographic elements can be exposed with various forms of energy which encompass the ultraviolet, visible, and infrared regions of the electromagnetic spectrum as well as with electron beam, beta radiation, gamma radiation, x-ray, alpha particle, neutron radiation, and other forms of corpuscular and wave-like radiant energy in either noncoherent (random phase) forms or coherent (in phase) forms, as produced by lasers. When the photographic elements are intended to be exposed by x-rays, they can include features found in conventional radiographic elements.

The photographic elements are preferably exposed to actinic radiation, typically in the visible region of the spectrum, to form a latent image, and then processed to form a visible image, preferably by other than heat treatment. Processing is preferably carried out in the known RA-4™ (Eastman Kodak Company) Process or other processing systems suitable for developing high chloride emulsions.

#### Photographic Grade Paper of Examples

A photographic paper support was produced by refining a pulp furnish of 50% bleached hardwood kraft, 25% bleached hardwood sulfite, and 25% bleached softwood sulfite through a double disk refiner, then a Jordan conical refiner to a Canadian Standard Freeness of 200 cc. To the resulting pulp furnish was added 0.2% alkyl ketene dimer, 1.0% cationic cornstarch, 0.5% polyamide-epichlorohydrin, 0.26% anionic polyacrylamide, and 5.0% TiO<sub>2</sub> on a dry weight basis. An about 46.5 lbs. per 1000 sq. ft. (ksf) bone dry weight base paper was made on a fourdrinier paper machine, wet pressed to a solid of 42%, and dried to a

moisture of 10% using steam-heated dryers achieving a Sheffield Porosity of 160 Sheffield Units and an apparent density 0.70 gm/cc. The paper base was then surface sized using a vertical size press with a 10% hydroxyethylated cornstarch solution to achieve a loading of 3.3 wt. % starch. The surface sized support was calendered to an apparent density of 1.04 grm/cc, and a thickness of 122  $\mu$ m.

The following examples illustrate the practice of this invention. They are not intended to be exhaustive of all possible variations of the invention. Parts and percentages are by weight unless otherwise indicated.

## EXAMPLES

### Example 1

The following laminated photographic paper bases (samples 1 through 6) were prepared by extrusion laminating the following sheets to both sides of a photographic grade cellulose paper support:

#### Bottom Sheet

BICOR 70MLT (Mobil Chemical Co.)

A one-side matte finish, one-side treated polypropylene sheet (18  $\mu$ m thick, d=0.9 g/cc) consisting of a solid oriented polypropylene core. The bottom sheet was extrusion laminated to a photographic grade cellulose paper support with a clear polyolefin adhesive (22.5 g/m<sup>2</sup>) with the matte finish side on the outside.

#### Paper Base

The paper support was 25% thinner than normal (122  $\mu$ m instead of 160  $\mu$ m) and had no TiO<sub>2</sub> included as is normally used for standard photographic base to obtain adequate optical properties; this was possible because of the beneficial effects of the invention.

#### Top Sheet (Emulsion Side)

A composite sheet consisting of 5 layers identified as L1, L2, L3, L4, and L5. L1 is the layer on the outside of the package to which the photosensitive silver halide layer was attached. L6 was the extrusion coated adhesive layer used to laminate the top sheet to the paper support.

The top sheet was coextruded and biaxially oriented. L6 was not part of this coextruded and biaxially oriented film.

Variations in L2, L3, L4, and L5 were made to demonstrate improvements in optical performance of a photographic nature. FIG. 1 shows the explanation for the sample design. Coating Format 1 below was utilized to coat samples #1-#6 with a silver halide emulsion.

| Coating Format 1                   | Laydown mg/m <sup>2</sup> |
|------------------------------------|---------------------------|
| <u>Layer Blue Sensitive Layer</u>  |                           |
| Gelatin                            | 1300                      |
| Blue sensitive silver              | 200                       |
| Y-1                                | 440                       |
| ST-1                               | 440                       |
| A-1                                | 190                       |
| <u>Layer Interlayer</u>            |                           |
| Gelatin                            | 650                       |
| SC-1                               | 55                        |
| S-1                                | 160                       |
| <u>Layer Green Sensitive Layer</u> |                           |
| Gelatin                            | 1100                      |
| Green sensitive silver             | 70                        |
| M-1                                | 270                       |
| S-1                                | 75                        |
| S-2                                | 32                        |

-continued

| Coating Format 1                 | Laydown mg/m <sup>2</sup> |    |
|----------------------------------|---------------------------|----|
| ST-2                             | 20                        | 5  |
| ST-3                             | 165                       |    |
| ST-4                             | 530                       |    |
| <u>Layer UV Interlayer</u>       |                           |    |
| Gelatin                          | 635                       |    |
| UV-1                             | 30                        | 10 |
| UV-2                             | 160                       |    |
| SC-1                             | 50                        |    |
| S-3                              | 30                        |    |
| S-1                              | 30                        |    |
| <u>Layer Red Sensitive Layer</u> |                           |    |
| Gelatin                          | 1200                      | 15 |
| Red sensitive silver             | 170                       |    |
| C-1                              | 365                       |    |
| S-1                              | 360                       |    |
| UV-2                             | 235                       |    |
| S-4                              | 30                        | 20 |
| SC-I                             | 3                         |    |
| <u>Layer UV Overcoat</u>         |                           |    |
| Gelatin                          | 440                       |    |
| UV-1                             | 20                        |    |
| UV-2                             | 110                       | 25 |
| SC-1                             | 30                        |    |
| S-3                              | 20                        |    |
| S-1                              | 20                        |    |
| <u>Layer SOC</u>                 |                           |    |
| Gelatin                          | 490                       | 30 |
| SC-1                             | 17                        |    |
| SiO <sup>2</sup>                 | 200                       |    |
| Surfactant                       | 2                         |    |

## APPENDIX



ST-1 = N-tert-butylacrylamide/n-butyl acrylate copolymer (50:50)  
 S-1 = dibutyl phthalate



S-2 = diundecyl phthalate

-continued

ST-2



S-3 = 1,4-Cyclohexyldimethylene bis(2-ethylhexanoate)

C-1



S-4 = 2-(2-Butoxyethoxy)ethyl acetate

Dye 1



65

FIGURE 1



Table 1 lists the characteristics of the layers that were held constant for these examples.

TABLE 1

| Layer | Material                                    | Thickness, microns |
|-------|---------------------------------------------|--------------------|
| L1    | LD Polyethylene with red and blue colorants | 0.762              |
| L2    | Polypropylene                               | 4.2                |
| L3    | Voided Polypropylene                        | 24.9               |
| L4    | Polypropylene                               | 4.32               |
| L5    | Polypropylene                               | 0.762              |

The L3 layer is microvoided and further described in Table 2 where the refractive index and geometrical thickness is shown for measurements made along 15 slices. The term "slice" does not imply continuous layers; a slice along another location would yield different but approximately the same thicknesses. The sublayer areas (slices) with a refractive index of 1 are voids that are filled with air, and the remaining slices (layers) are polypropylene between the voids.

TABLE 2

| Sublayer (slice) of L3 | Refractive Index | Thickness, $\mu\text{m}$ |
|------------------------|------------------|--------------------------|
| 1                      | 1.49             | 2.54                     |
| 2                      | 1                | 1.527                    |
| 3                      | 1.49             | 2.79                     |
| 4                      | 1                | 1.016                    |
| 5                      | 1.49             | 1.778                    |
| 6                      | 1                | 1.016                    |
| 7                      | 1.49             | 2.286                    |
| 8                      | 1                | 1.016                    |
| 9                      | 1.49             | 2.032                    |
| 10                     | 1                | 0.762                    |
| 11                     | 1.49             | 2.032                    |
| 12                     | 1                | 1.016                    |
| 13                     | 1.49             | 1.778                    |
| 14                     | 1                | 1.016                    |
| 15                     | 1.49             | 2.286                    |

Table 3 lists the variations of  $\text{TiO}_2$  amounts (weight %) in layers L2 through L5 for each sample.

TABLE 3

|          | L2 $\text{TiO}_2$<br>% by wt | L3 $\text{TiO}_2$<br>% by wt | L4 and L5 $\text{TiO}_2$<br>% by wt |
|----------|------------------------------|------------------------------|-------------------------------------|
| 5        | 4                            | 4                            | 0                                   |
| 10       | 4                            | 4                            | 18                                  |
| Sample 3 | 4                            | 11                           | 0                                   |
| Sample 4 | 4                            | 11                           | 18                                  |
| Sample 5 | 11                           | 11                           | 18                                  |
| Sample 6 | 11                           | 11                           | 0                                   |

TABLE 4

|          | MTF 2 | opacity | L STAR UVO |
|----------|-------|---------|------------|
| Sample 1 | 68    | 90.02   | 92.29      |
| Sample 2 | 64    | 91.52   | 93.16      |
| Sample 3 | 73    | 91.89   | 93.31      |
| Sample 4 | 70    | 91.59   | 93.52      |
| Sample 5 | 71    | 93.01   | 93.42      |
| Sample 6 | 78    | 92.45   | 93.57      |

Table 4 lists the measured properties of each sample; MTF 2 cycle/mm sharpness ratings, opacity, and LSTAR lightness values for the examples. Some of this data was gathered from photographic emulsion coated samples made from each example. The results show that the choice of layer thickness, composition and  $\text{TiO}_2$  loading have a major effect on the photographic performance properties. Additionally, the amount of change is remarkable with such relatively thin layers with very low amounts of  $\text{TiO}_2$ , compared to prior art. The LSTAR values are remarkable in that they all exceed standard photographic products. The OPACITY is low but it can easily be improved with a pigmented tie layer or  $\text{TiO}_2$  additions in the raw paper base.

The beneficial effects of a voided L3 layer with a clear L4 and L5 layers can be demonstrated with the sharpness data. In each case of paired samples (Tables 5 through 7), the higher sharpness is obtained with the  $\text{TiO}_2$  removed from the L4 and L5 layer, not an expected result. This is an effect of the optical performance provided by the voided L3 layer which appears to work better for sharpness when there is no pigmentation below it.

TABLE 5

|          | L2 $\text{TiO}_2$<br>% by wt | L3 $\text{TiO}_2$<br>% by wt | L4 and L5 $\text{TiO}_2$<br>% by wt | MTF 2 |
|----------|------------------------------|------------------------------|-------------------------------------|-------|
| 55       | 4                            | 4                            | 0                                   | 68    |
| Sample 2 | 4                            | 4                            | 18                                  | 64    |

TABLE 6

|          | L2 $\text{TiO}_2$<br>% by wt | L3 $\text{TiO}_2$<br>% by wt | L4 and L5 $\text{TiO}_2$<br>% by wt | MTF 2 |
|----------|------------------------------|------------------------------|-------------------------------------|-------|
| 60       | 4                            | 11                           | 0                                   | 73    |
| Sample 4 | 4                            | 11                           | 18                                  | 70    |

TABLE 7

|          | L2 TiO <sub>2</sub><br>% by wt | L3 TiO <sub>2</sub><br>% by wt | L4 and L5 TiO <sub>2</sub><br>% by wt | MTF 2 |
|----------|--------------------------------|--------------------------------|---------------------------------------|-------|
| Sample 6 | 11                             | 11                             | 0                                     | 78    |
| Sample 5 | 11                             | 11                             | 18                                    | 71    |

The invention has been described in detail with particular reference to preferred embodiments thereof, but it will be understood that variations and modifications can be effected within the spirit and scope of the invention.

We claim:

1. A photographic element comprising a paper base, at least one photosensitive silver halide layer, a layer of biaxially oriented polyolefin sheet between said paper base and said silver halide layer, wherein said biaxially oriented polyolefin sheet comprises an upper layer that comprises between 4 and 24% of a white pigment; and adjacent said upper layer a core layer that is microvoided; and adjacent and back of said core layer a layer of polyolefin that is substantially colorant and pigment free.
  2. The photographic element of claim 1 wherein said core layer comprises between 2 and 18% of white pigment.
  3. The photographic element of claim 1 wherein the upper surface of said biaxially oriented sheet comprises a skin layer that is substantially pigment free.
  4. The photographic element of claim 1 wherein said biaxially oriented sheet further comprises on the lower side of said substantially colorant free layer a layer comprising white pigment.
  5. The photographic element of claim 1 wherein on the lower side of said biaxially oriented sheet there is a binder layer comprising white pigment.
  6. The photographic element of claim 1 wherein said white pigment comprises titanium dioxide.
  7. The photographic element of claim 1 wherein said upper layer is between about 1 to 15  $\mu\text{m}$  in thickness.
- 10
8. The photographic element of claim 1 wherein said microvoided core layer is between about 10 and 60  $\mu\text{m}$  in thickness.
  9. The photographic element of claim 1 wherein the substantially colorant free layer adjacent said microvoided layer is between about 2 and 15  $\mu\text{m}$  in thickness.
  10. The photographic element of claim 1 wherein said upper layer comprises between 15 and 20 weight percent of white pigment.
  11. The photographic element of claim 1 wherein said microvoided layer comprises between 2 and 8 weight percent of white pigment.
  12. The photographic element of claim 1 wherein said paper comprises cellulose fibers.
  13. The photographic element of claim 12 further comprising a biaxially oriented polymer sheet on the bottom side of said element in back of said paper.
  14. The photographic element of claim 13 wherein said biaxially oriented polyolefin sheet comprises an upper surface layer comprising blue colorant.
  15. The photographic element of claim 13 wherein said biaxially oriented polyolefin sheet comprises polypropylene.
  16. The photographic element of claim 13 wherein said biaxially oriented sheet on the bottom side of said element comprises polypropylene.
  17. The photographic element of claim 13 wherein said at least one photosensitive silver halide layer comprises a cyan dye image-forming unit, a magenta dye image-forming unit, and a yellow dye image-forming unit.
  18. The photographic layer of claim 1 wherein said core layer that is microvoided further comprises white pigment.
  19. The photographic element of claim 14 wherein said core layer comprises between 2 and 18% of white pigment.
  20. The photographic element of claim 13 wherein said microvoided core layer is between about 10 and 60  $\mu\text{m}$  in thickness.
- 15
- 20
- 25
- 30
- 35

\* \* \* \* \*